

## UNITED STATES PATENT OFFICE.

ALFRED L. BROADBENT, OF WILMINGTON, DELAWARE, ASSIGNOR TO E. I. DU PONT DE NEMOURS & COMPANY, OF WILMINGTON, DELAWARE, A CORPORATION OF DELAWARE.

METHOD OF PREPARING SHORT-FIBER CELLULOSIC MATERIAL FOR CHEMICAL TREATMENT.

No Drawing.

Application filed November 8, 1919. Serial No. 336,719.

To all whom it may concern:

Be it known that I, ALFRED L. BROADBENT, a citizen of the United States, and a resident of Wilmington, in the county of New Castle and State of Delaware, have invented a certain new and useful Method of Preparing Short-Fiber Cellulosic Material for Chemical Treatment, of which the following is a specification.

10 This invention relates to the preparation of short-fiber cellulosic material to render it amenable to a chemical treatment designed to convert it into certain of its derivatives; while not restricted thereto the invention is 15 particularly applicable to the preparation of wood pulp for nitration, and therefore I describe it with particular reference to that art.

In order to obtain a uniformly nitrated 20 nitrocellulose from any fibrous material, it is essential that the material be in such physical condition that the nitrating acids will completely penetrate the individual fibers. If the fibrous material contains hard compact 25 lumps, or is otherwise incompletely opened up, the nitrating acid has to penetrate these hard lumps and the like, instead of having easy and immediate access to all the fibers, and as it penetrates the lumps, the 30 acid becomes gradually weaker in nitric acid as this acid is used up in nitration. The weakened acid that penetrates to the interior of the lump has a marked hydrolyzing action on the cellulose, and therefore leads to the 35 production of nitrated compounds of obscure composition which differ from nitrocellulose in being gelatinous in nature, and which exhibit chemical and physical characteristics different from those of true nitrocellulose. 40 If the lumps are exceedingly compact, some of the fiber may even resist nitration entirely. The result of using material containing these lumps is the production of nitrated material which is non-uniformly nitrated to 45 such an extent as to be decidedly inferior, or indeed unsuitable, for use for purposes of colloidization or solution.

The difficulty in obtaining the fibers 50 opened up sufficiently to permit the nitrating acid to freely and uniformly penetrate the individual fibers is especially characteristic of wood pulp. If dried in bulk, the dried

pulp will contain hard, compact lumps of fiber which cannot be readily opened up to a condition in which the nitrating acid will 55 freely penetrate them. In sheet form, also, wood pulp exhibits a tendency to dry in a condition that prevents the uniform penetration of the nitrating acid. A further objection to the use of wood pulp for nitration 60 lies in the tendency of the fiber, owing to its shortness, to be carried along in excessive amounts with the spent acid recovered from the nitration operation whereby the entrained pulp causes the rapid filling up of 65 the spent acid filters, and entails other operating difficulties; entrained pulp also occasions losses in the washing processes in the 70 purification treatment subsequent to nitration.

I have devised a method of so preparing short-fiber cellulosic material that the resulting material will not dry in lumps, but on the contrary, after picking will dry to a fluffy form free from hard lumps and of such character that the nitrating acid will readily and uniformly penetrate the individual fibers, thereby yielding a uniformly nitrated nitrocellulose.

In general my invention consists in the 80 matters hereinafter described and claimed, it being understood that I do not restrict it either to the art of nitration or to the treatment of wood pulp, but for the sake of definiteness and brevity describe it with more particular reference to the art of nitrating wood pulp.

My invention comprises blending wood pulp, which has a relatively short fiber, with cotton in any unspun form, the cotton having a relatively longer fiber than the wood pulp, this blending being done previous to the operations of teasing or picking and drying which precede nitration. The longer-fiber cotton in intimate mixture with the short-fiber wood pulp prevents the drying of the wood pulp into hard compact lumps and gives a mixture that, after passing through a teasing or picking machine, will dry to a fluffy form free from hard lumps, with the fiber opened up sufficiently to permit the nitrating acid to freely and uniformly penetrate all the individual fibers, so that, upon nitration, a superior and uniformly nitrated 90 95 100

nitrocellulose is produced. Also, the various difficulties that would ordinarily be met with, and losses that would ordinarily be sustained because of the tendency of wood

5 pulp to penetrate the holes in the apparatus used in the nitrating and purifying operations, are greatly minimized.

In proceeding in accordance with my invention, I prefer to use a mixture of equal 10 parts of cotton fiber and wood pulp, but can secure the desired results with as low as forty per cent cotton fiber to sixty per cent wood pulp. Of course, mixtures having a larger percentage of cotton fiber can be used

15 if desired. There is no restriction as to the particular grades of cotton fiber which can be used. I have found, however, that the most satisfactory results are obtained either with cotton linters, or with a mixture of cotton 20 linters with another or other grades of cotton fiber in which mixture the amount of cotton linters is at least fifty per cent of the total amount of cotton fiber present. The nitrocellulose resulting from the nitration 25 of cotton is in no way objectionable for the purposes for which the nitrated material is used.

To obtain the desired uniformity in the mixture, it is necessary to thoroughly separate the fibers of the wood pulp, preferably 30 by steeping in water. The wood pulp may be charged with the crude cotton into a digester and submitted to the purification treatment accorded to the cotton, or it may 35 be added to the cotton at any subsequent operation as in the bleaching or washing operations, provided there is agitation sufficient to intimately blend the two materials. After squeezing out the bulk of the water 40 from the mixture of wood pulp and cotton, and passing the material through a teasing or picking machine, the mixture is dried,

giving, as before stated, a fluffy form free from hard lumps and so forth. The material so prepared may then be nitrated in any 45 usual or preferred way.

Having thus described my invention, I claim:—

1. In the conversion of short-fiber cellulosic material into esters thereof, the method 50 which comprises mixing with such material a different longer-fiber cellulosic material.

2. In the conversion of short-fiber cellulosic material into esters thereof, the method 55 which comprises adding to such material a longer-fiber cellulosic material.

3. In the conversion of wood pulp into certain derivatives thereof, the method 60 which comprises mixing cotton fiber with the wood pulp.

4. In the nitration of wood pulp, the method which comprises mixing cotton fiber with the wood-pulp.

5. In the nitration of wood pulp, the method 65 which comprises mixing with the wood pulp substantially an equal quantity of cotton fiber.

6. In the conversion of short-fiber cellulosic material into esters thereof, the method 70 which comprises adding to the material a cellulosic longer-fiber material, agitating the materials with liquid thereby to intimately mix them, removing the bulk of the liquid, separating the fibers of the mixture, and drying.

7. In the nitration of wood pulp, the method which comprises adding cotton fiber to the pulp, agitating the pulp and cotton fiber with water thereby to intimately mix them, removing the bulk of the water, separating the fibers of the mixture, and drying.

In testimony whereof I affix my signature.

ALFRED L. BROADBENT.